

1

3,657,411  
TWO-STAGE DRAWING PROCESS FOR POLY-  
BENZIMIDAZOLE FIBER

Thomas C. Bohrer, Charlotte, N.C., and David H. T. Chen, Wilmington, Del., assignors to Celanese Corporation, New York, N.Y.  
No Drawing. Continuation-in-part of application Ser. No. 770,083, Oct. 23, 1968. This application Sept. 15, 1970, Ser. No. 72,535

Int. Cl. D02j 1/22  
U.S. CL. 264—290 R

11 Claims

### ABSTRACT OF THE DISCLOSURE

Polybenzimidazole fiber is drawn in two-stages where in the second draw is at a lower temperature than the first. After double drawing the tenacity and initial modulus of the fiber are higher than after the first stage draw. The first stage draw may be effected at a temperature in the range 300–650° C. with a ratio of 1.5–3.5× while the second stage draw may be conducted at a lower temperature in the range 200–500° C. with a ratio of 1.05–1.5×. Various means of heating are disclosed, including radiation and contact with hot metal surfaces. Exposure time is disclosed to be a function of the mode of heating and the temperature used.

### CROSS-REFERENCE TO RELATED APPLICATION

This is a continuation-in-part of our co-pending U.S. Ser. No. 770,083, filed Oct. 23, 1968.

### BACKGROUND OF THE INVENTION

Double drawing, that is, two stage drawing, of polymer fibers or filaments is a well known method for increasing tensile properties, particularly tenacity. Heretofore, however, the second draw has been conducted at a higher temperature than that employed in the first draw, especially when working with high molecular weight polymers such as nylons, polyesters, and polyolefins. See, for instance, U.S. Pat. Nos. 2,556,295 to Pace and 3,400,194 to Boone et al. which disclose two stage polyester hot drawing processes, the second stage of which is conducted at more severe conditions than the first stage. It was thought that these high molecular weight polymer fibers needed a more severe second draw treatment because of their increased stiffness after the first draw.

It is an object of the present invention to provide a process for improving the tensile properties of polybenzimidazole fiber.

It is another object of the invention to provide an improved two stage hot drawing process for polybenzimidazole fiber.

These and other objects, as well as the scope, nature and utilization of the process will be apparent from the following detailed description and appended claims.

### SUMMARY OF THE INVENTION

It has been found that a process for improving the tensile properties of polybenzimidazole fiber comprises subjecting the fiber to a first draw treatment at a temperature in the range of from 300 to 650° C. and at a draw ratio in the range of from 1.5:1 to 3.5:1, and thereafter subjecting the resulting drawn fiber to a second draw treatment at a draw ratio in the range of from 1.05:1 to 1.5:1 and at a temperature which is lower than that used in the first draw and which is within the range of from 200 to 500° C. to produce a polybenzimidazole fiber product having a higher tenacity and higher initial modulus than that of the fiber product obtained from the first draw treatment.

2

### DESCRIPTION OF PREFERRED EMBODIMENTS

#### The starting polymer

Polybenzimidazoles are a known class of heterocyclic polymers, which consist essentially of recurring units of the following Formulas I and II.

Formula I is:



wherein R is a tetravalent aromatic nucleus, with the nitrogen atoms forming the benzimidazole rings being paired upon adjacent carbon atoms, i.e., ortho carbon atoms, of the aromatic nucleus, and R' is a member of the class consisting of an aliphatic (alkylene) group, a cycloaliphatic ring, an aromatic ring and a heterocyclic ring such as pyridine, pyrazine, furan, quinoline, thiophene, and pyran.

Formula II is:



wherein Z is an aromatic nucleus having the nitrogen atoms forming the benzimidazole ring paired upon adjacent carbon atoms of the aromatic nucleus.

Preferably, aromatic polybenzimidazoles are used in the present invention, that is, fibers prepared from polymers consisting essentially of the recurring units of Formula II and Formula I wherein R' is an aromatic ring or a heterocyclic ring.

As set forth in U.S. Pat. No. 3,174,947 and U.S. Reissue Pat. No. 26,065, which are incorporated herein by reference, the aromatic polybenzimidazoles having the recurring units of Formula II may be prepared by self-condensing a trifunctional aromatic compound containing only a single set of ortho disposed diamino substituents and an aromatic, preferably phenyl, carboxylate ester substituent. Exemplary of polymers of this type is poly-2,5(6)-benzimidazole prepared by the auto-condensation of phenyl-3,4-diaminobenzoate.

As also set forth in the above-mentioned patents, the aromatic polybenzimidazoles having the recurring units of Formula I may be prepared by condensing an aromatic tetraamine compound containing a pair of ortho-diamino substituents on the aromatic nucleus with a dicarboxyl compound selected from the class consisting of (a) the diphenyl ester of an aromatic dicarboxylic acid, (b) the diphenyl ester of a heterocyclic dicarboxylic acid wherein the carboxyl groups are substituents upon carbon in a ring compound selected from the class consisting of pyridine, pyrazine, furan, quinoline, thiophene and pyran and (c) an anhydride of an aromatic dicarboxylic acid.

Examples of aromatic polybenzimidazoles which have the recurring structure of Formula I and which may be formed into fibers and subjected to the double drawing process of the present invention include:

poly-2,2' (m-phenylene) 5,5'-bibenzimidazole;  
poly-2,2'-(pyridylene-3'',5'')-5,5'-bibenzimidazole;  
poly-2,2'-(furylene-2'',5'')-5,5'-bibenzimidazole;  
poly-2,2'-(naphthalene-1'',6'')-5,5'-bibenzimidazole;  
poly-2,2'-(biphenylene 4'',4'')-5,5'-bibenzimidazole;  
poly-2,6-(m-phenylene)-diimidazobenzene;  
poly-2,2' (m-phenylene)-5,5'-di(benzimidazole) ether;  
poly-2,2' (m-phenylene)-5,5'-di(benzimidazole) sulfide;  
poly-2,2' (m-phenylene)-5,5'-di(benzimidazole) sulfone;

## 3

poly-2',2' (m-phenylene)-5,5'-di(benzimidazole) methane; poly-2',2" (m-phenylene)-5',5"-di(benzimidazole) propane-2,2; and poly-2',2" (m-phenylene)-5',5" di(benzimidazole) ethylene-1,2

where the double bonds of the ethylene groups are intact in the final polymer.

The preferred aromatic polybenzimidazole fiber is one prepared from poly-2,2'-(m-phenylene)-5,5'-bibenzimidazole, the recurring unit of which is:



Any polymerization process known to those skilled in the art may be employed to prepare the polybenzimidazole which may then be spun into fiber and subjected to the double drawing process of the present invention. With respect to aromatic polybenzimidazoles, preferably, equimolar quantities of the monomeric tetraamine and dicarboxyl compound are introduced into a first stage melt polymerization reaction zone and heated therein at a temperature above about 200° C., preferably at least 250° C., and more preferably from about 270 to 300° C. The reaction is conducted in a substantially oxygen-free atmosphere, i.e., below about 20 p.p.m. oxygen and preferably below about 8 p.p.m. oxygen, until a foamed prepolymer is formed. Usually, the first stage reaction is continued until a prepolymer is formed having an inherent viscosity, expressed as deciliters per gram, of at least 0.1, and preferably from about 0.13 to 0.3, the inherent viscosity (I.V.) as used in the present specification and claims being determined from a solution of 0.4 gram of the polymer in 100 ml. of 97 percent H<sub>2</sub>SO<sub>4</sub> at 25° C.

After the conclusion of the first stage reaction, which normally takes at least 0.5 hour and preferably 1 to 3 hours, the foamed prepolymer is cooled and then powdered or pulverized in any convenient manner. The resulting prepolymer powder is then introduced into a second stage polymerization reaction zone wherein it is heated under substantially oxygen-free conditions, as described above, to yield a polybenzimidazole polymer product, desirably having an I.V., as measured above, of at least 0.6 e.g., 0.80 to 1.1 or more.

The temperature employed in the second stage is at least 250° C., preferably at least 325° C., and more preferably from about 350 to 425° C. The second stage reaction generally takes at least 0.5 hour, and preferably from about 1 to 4 hours or more.

#### Preparation of the fiber

As is well known, the polybenzimidazoles are generally formed into fibers or filaments by dry or wet spinning a solution of the polymer in an appropriate solvent such as dimethylacetamide, dimethylformamide, dimethylsulfoxide or sulfuric acid through an opening of predetermined shape into an evaporative atmosphere for the solvent in which most of it is evaporated, or into a coagulation bath, resulting in the polymer having the desired shape.

The polymer solutions may be prepared, for example, by dissolving sufficient polybenzimidazole in the solvent to yield a final solution suitable for extrusion containing from about 10 to 45 percent by weight of polymer, based on the total weight of the solution, preferably from about 20 to 30 percent by weight.

One suitable means for dissolving the polymer in the solvent is by mixing the materials at a temperature above the atmospheric boiling point of the solvent, for example, 25 to 120° C. above such boiling point, and at a pressure of 2 to 15 atmospheres for a period of 1 to 5 hours.

Preferably, the above polymer solutions, after suitable

## 4

filtration to remove any undissolved portions, are dry spun. For example, the solutions may be extruded through a spinneret into a conventional type downdraft spinning column containing a circulating inert gas such as nitrogen, noble gases, combustion gases or super heated steam. Conveniently, the spinneret face is at a temperature of from 130 to 170° C., the top of the column from about 120 to 220° C., the middle of the column from about 140 to 250° C., and the bottom of the column from about 60 to 320° C. After leaving the spinning column, the fibers are taken up, at a speed in the range of from about 50 to 350 meters per minute, washed thoroughly such as with water in order to remove residual solvent, and then dried in any suitable type of apparatus at a temperature in the range of from about 150 to 300° C. for about 2 to 100 hours or more.

Prior to being washed the dry-spun fibers are subjected to a slight steam drawing treatment at a draw ratio of from about 1.1:1 to 1.5:1.

This pre-wash drawing treatment is to be distinguished from the post-wash double drawing process of the present invention.

The present invention is directed to the post-wash drawing of the polybenzimidazole fibers and not their initial formation; therefore, any of the known methods for preparing the fibers in addition to those described above may be used.

#### First and second drawing stages

The resulting washed and dried polybenzimidazole fiber, preferably aromatic polybenzimidazole fiber, is then drawn (first draw) at a temperature in the range of about 300 to 650° C. at a draw ratio in the range of 1.5:1 to 3.5:1, and thereafter is drawn (second draw) at a temperature lower than that used in the first draw which is in the range of from about 200 to 500° C. at a draw ratio of about 1.05:1 to 1.5:1 to produce a polybenzimidazole fiber product having a higher tenacity and higher initial modulus than that of the fiber product obtained from the first draw treatment.

The first draw treatment is preferably conducted at a temperature in the range of 450 to 600° C., and the second draw treatment is preferably conducted at a temperature in the range of 390 to 470° C. which is below that used in the first draw treatment.

The first draw treatment is preferably conducted at a draw ratio of 2.0:1 to 3.2:1, and the second draw treatment is preferably conducted at a draw ratio of about 1.1:1 to 1.3:1.

The manner in which heat is applied to the polybenzimidazole fiber undergoing hot drawing may be varied widely. For instance, the fiber may be heated via radiation heating by passage through a muffle furnace or other hot gas heating zone. Alternatively, the polybenzimidazole fiber undergoing hot drawing may be heated via conductive heating wherein the fiber is passed over a hot surface, such as one or more hot shoe, roll, plate, pin, etc.

As will be apparent to those skilled in the art, the residence time during which the fiber is being drawn at the elevated temperature indicated varies with the mode of heating selected. For instance, a generally longer residence time is commonly utilized when the mode of heating is via radiation, than when the mode of heating is via conduction.

When the mode of heating is via radiation, the first draw treatment residence times commonly range from about 5 to 30 seconds (preferably 10 to 20 seconds), and the second draw treatment residence times commonly range from about 1 to 20 seconds (preferably 3 to 15 seconds). When the mode of heating is via conduction, the first draw treatment residence times commonly range from about 0.2 to 3 seconds (preferably 0.3 to 1 second), and second raw treatment residence times commonly range from about 0.1 to 1.5 seconds (preferably 0.2 to 0.8 second). The exact residence time selected for

optimum results will also be influenced by the temperature of the draw treatment as will be apparent to those skilled in the art.

As previously mentioned, the essence of the present invention is the discovery that the second draw treatment can be advantageously conducted at milder conditions and not more strenuous or severe conditions as would be expected. Not only can the second draw be

treatment (post-wash draw) by drawing it in a muffle furnace maintained at a temperature of 550° C. The draw ratio used was 2.2:1 and the residence time of the yarn in the furnace was 12 seconds.

This "intermediate" drawn fiber was then used as the feed fiber to a second rawing stage in the muffle furnace, wherein the temperature and draw ratio were varied as shown in Table I below.

TABLE I

| Experiment Number                            | Residence time in seconds | Draw ratio <sup>1</sup> | Supply roll rate, meters/minute | Temperature in degrees centigrade | Percent of draw break <sup>2</sup> | Denier per fiber | Elongation, percent <sup>3</sup> | Tenacity, grams/denier | Initial modulus, grams/denier |
|----------------------------------------------|---------------------------|-------------------------|---------------------------------|-----------------------------------|------------------------------------|------------------|----------------------------------|------------------------|-------------------------------|
| I. Feed fiber from first stage draw          |                           |                         |                                 |                                   |                                    |                  |                                  |                        |                               |
|                                              | 12                        | 2.2                     | 55                              | 550                               | 60                                 | 4.2              | 31                               | 5.1                    | 28                            |
| II. Second stage draw conditions and results |                           |                         |                                 |                                   |                                    |                  |                                  |                        |                               |
| 1                                            | 7                         | 1.21                    | 55                              | 560                               | 40                                 | 3.5              | 29                               | 2.9                    | 15                            |
| 2                                            | 7                         | 1.32                    | 55                              | 560                               | 60                                 | 3.1              | 25                               | 3.4                    | 17                            |
| 3                                            | 7                         | 1.42                    | 55                              | 560                               | 80                                 | 2.8              | 19                               | 2.8                    | 12                            |
| 4                                            | 7                         | 1.41                    | 55                              | 530                               | 40                                 | 3.0              | 16                               | 3.3                    | 13                            |
| 5                                            | 7                         | 1.61                    | 55                              | 530                               | 60                                 | 2.7              | 14                               | 3.7                    | 14                            |
| 6                                            | 7                         | 1.71                    | 55                              | 500                               | 60                                 | 2.6              | 9                                | 4.5                    | 14                            |
| 7                                            | 7                         | 1.93                    | 55                              | 500                               | 80                                 | 2.1              | 6                                | 4.9                    | 12                            |
| 8                                            | 7                         | 1.16                    | 55                              | 470                               | 40                                 | 3.3              | 17                               | 5.9                    | 24                            |
| 9                                            | 7                         | 1.25                    | 55                              | 470                               | 60                                 | 3.2              | 12                               | 5.7                    | 20                            |
| 10                                           | 7                         | 1.14                    | 55                              | 440                               | 40                                 | 3.7              | 16                               | 5.7                    | 23                            |
| 11                                           | 7                         | 1.19                    | 55                              | 440                               | 55                                 | 3.4              | 12                               | 6.6                    | 23                            |
| 12                                           | 7                         | 1.24                    | 55                              | 440                               | 70                                 | 3.3              | 9                                | 6.9                    | 21                            |
| 13                                           | 7                         | 1.09                    | 55                              | 425                               | 25                                 | 3.8              | 23                               | 5.4                    | 26                            |
| 14                                           | 7                         | 1.14                    | 55                              | 425                               | 40                                 | 3.3              | 13.2                             | 5.9                    | 22                            |
| 15                                           | 7                         | 1.19                    | 55                              | 425                               | 55                                 | 3.2              | 10                               | 6.4                    | 21                            |
| 16                                           | 7                         | 1.24                    | 55                              | 425                               | 70                                 | 3.1              | 8                                | 7.1                    | 20                            |

<sup>1</sup> The draw ratio is the rate at which the stretch roll or take-up roll is rotated divided by the rate of rotation of the supply or feed roll.

<sup>2</sup> Draw break is the draw ratio at which the yarn breaks.

<sup>3</sup> Measured at the breakpoint of the yarn.

<sup>4</sup> "TEV" = Index of fiber organization wherein T is tenacity at break in grams per denier and E is elongation of percent extension from original length at break in tensile test. An explanation of this test and its significance is given in the Textile Research Journal 36, No. 7, pages 593-602, July 1966.

<sup>5</sup> Stress of tangent of initial slope at 2% elongation extended to 100% elongation. Is measure of stiffness in the elastic region and in the region of use.

conducted at a lower temperature within the range of 200 to 500° C., but a lower draw ratio and residence time may also be employed to produce a polybenzimidazole fiber product having a higher tenacity and initial modulus values than the intermediate product fiber obtained from the first draw. The use of the milder or less severe conditions in the second draw treatment to obtain the improved tensile properties is completely contrary to known high molecular weight polymer fiber drawing technology with respect to two stage drawing.

The drawing operation (first and second drawing treatments or stages) may be conducted on a batch, continuous or semi-continuous basis, and preferably is conducted on a continuous basis.

The present invention is equally applicable to the drawing of mono- or multi-filaments or fibers, for example, yarns having 10 to 1000 filaments or more. The denier of the fiber used in the present invention is not critical, commonly being from about 1 to 20 denier per fiber (D.P.F.).

The following examples are given as specific illustrations of the unexpected results achieved when practicing the process of the present invention.

#### EXAMPLE 1

Poly-2,2'-(m-phenylene) - 5,5' - bibenzimidazole (prepared by the polymerization of 3,3' - diaminobenzidine and diphenyl isophthalate) was dissolved in dimethyl acetamide. The resulting polymer solution (23 percent by weight solids) was extruded through a 50 hole spinneret into a downdraft spinning column containing circulating nitrogen to produce a 50 filament yarn of 400 total denier.

After leaving the spinning column, the yarn was taken up at a speed of 100 meters per minute and was then drawn (pre-wash draw) in steam at atmospheric pressure at a draw ratio of 1.1:1, washed with water on perforated bobbins and dried. The dried yarn had a tenacity of about 1.5 grams per denier and an elongation of about 100 percent.

The dried yarn was then subjected to a first drawing

As can be seen from the data of Table I, the less severe conditions used in the second stage draw treatment yield a polybenzimidazole yarn of increased tensile properties (i.e. tenacity and initial modulus). In Experiment Nos. 1, 2, and 3 the temperature of the second stage draw treatment (i.e. 560° C.) was in excess of that employed during the first stage draw treatment, and resulted in a decrease in both the tenacity and initial modulus values. In Experiment Nos. 4 and 5 the temperature of the second stage draw treatment (i.e. 530° C.) was less than that employed during the first stage draw treatment, but was still excessive. In Experiment Nos. 6, and 7 the second stage draw ratio was excessive, and the tenacity was decreased. Accordingly, Experiment Nos. 1 through 7 are presented for comparative purposes, and Experiment Nos. 8 through 16 are in accordance with applicants' improved process.

Similar results are obtained when a mono-filament polybenzimidazole is used in place of the yarn, as well as when other polybenzimidazole fibers or yarns such as those specifically mentioned heretofore are used.

#### EXAMPLE II

A washed and dried polybenzimidazole yarn [poly-2,2'-(m-phenylene)-5,5'-bibenzimidazole] substantially similar to that subjected to the drawing treatments of Example I was drawn via conductive heating rather than radiation heating. The yarn consisted of 50 continuous filaments and had a total denier of about 600. The yarn exhibited a single filament tenacity of about 1.7 grams per denier, an elongation of about 100 percent, and an initial modulus of about 38 grams per denier.

The yarn was subjected to a first drawing treatment (post-wash draw) by drawing while in moving contact with a pair of convex heated drawing shoes placed in an end-to-end relationship. Each drawing shoe had a length of 10 inches and a width of 1 1/4 inch, was resistance heated to the temperature indicated in Table II, and was provided with a smooth stainless steel alloy surface. During the first drawing treatment the drawing shoes were

maintained at 430° C. The draw ratio was 2.0:1, and the residence time of the yarn while in contact with the drawing shoes was about 1 second.

This "intermediate" drawn fiber was then used as the feed fiber to a second drawing stage on a pair of like drawing shoes at draw ratio of 1.2:1 and a contact time of about 0.6 second at various temperatures as shown in Table II.

TABLE II

| Experiment Number                            | Residence time in seconds | Draw ratio | Supply roll rate, meters/minute | Temperature in degrees centigrade | Denier per fiber | Elongation, percent | Tenacity, grams/denier | Initial modulus, grams/denier |
|----------------------------------------------|---------------------------|------------|---------------------------------|-----------------------------------|------------------|---------------------|------------------------|-------------------------------|
| I. Feed fiber from first draw                |                           |            |                                 |                                   |                  |                     |                        |                               |
|                                              | 1                         | 2.0        | 25                              | 430                               | 5.5              | 31.9                | 4.7                    | 26.2                          |
| II. Second stage draw conditions and results |                           |            |                                 |                                   |                  |                     |                        |                               |
| 1-----                                       | 0.6                       | 1.2        | 50                              | 460                               | 5.0              | 30.1                | 2.9                    | 16.0                          |
| 2-----                                       | 0.6                       | 1.2        | 50                              | 445                               | 5.1              | 33.0                | 3.6                    | 20.4                          |
| 3-----                                       | 0.6                       | 1.2        | 50                              | 430                               | 5.0              | 29.9                | 4.3                    | 23.2                          |
| 4-----                                       | 0.6                       | 1.2        | 50                              | 415                               | 5.0              | 25.6                | 4.5                    | 22.8                          |
| 5-----                                       | 0.6                       | 1.2        | 50                              | 400                               | 5.1              | 19.9                | 4.9                    | 21.7                          |
|                                              |                           |            |                                 |                                   |                  |                     |                        | 96                            |

As can be seen from the data of Table II, the less severe conditions used in the second stage draw treatment yield a polybenzimidazole fiber of generally tensile properties (i.e. tenacity and initial modulus). In Experiment Nos. 1 through 3 the temperature of the second stage draw treatment was excessive, and resulted in a

improved process the benefits of the present process are clearly apparent since both the final tenacity and the initial modulus values exceed those obtained after the first draw stage.

## EXAMPLE IV

Example II was repeated with the modifications indicated. The draw ratio during the first draw treatment

TABLE IV

| Experiment Number                            | Residence time in seconds | Draw ratio | Supply roll rate, meters/minute | Temperature in degrees centigrade | Denier per fiber | Elongation, percent | Tenacity, grams/denier | Initial modulus, grams/denier |
|----------------------------------------------|---------------------------|------------|---------------------------------|-----------------------------------|------------------|---------------------|------------------------|-------------------------------|
| I. Feed fiber from first draw                |                           |            |                                 |                                   |                  |                     |                        |                               |
|                                              | 0.7                       | 3.0        | 25                              | 430                               | 4.6              | 20.5                | 5.2                    | 23.4                          |
| II. Second stage draw conditions and results |                           |            |                                 |                                   |                  |                     |                        |                               |
| 1-----                                       | 0.3                       | 1.2        | 75                              | 445                               | 3.0              | 22.1                | 4.8                    | 22.7                          |
| 2-----                                       | 0.3                       | 1.2        | 75                              | 430                               | 2.9              | 13.8                | 4.7                    | 17.3                          |
| 3-----                                       | 0.3                       | 1.2        | 75                              | 415                               | 2.8              | 12.2                | 5.3                    | 18.5                          |
| 4-----                                       | 0.3                       | 1.2        | 75                              | 400                               | 3.0              | 8.7                 | 5.6                    | 16.4                          |
|                                              |                           |            |                                 |                                   |                  |                     |                        | 119                           |

decrease in both the tenacity and initial modulus values. In Experiment No. 4 the tenacity was decreased slightly while the initial modulus was enhanced. Experiment No. 5 indicates that both the tenacity and the initial modulus were enhanced, and is in accordance with applicants' improved process.

## EXAMPLE III

Example II was repeated with the modifications indicated. The draw ratio during the first draw stage was 3.0:1, and the residence time while in contact with the first stage drawing shoes was about 0.7 second.

This "intermediate" drawn fiber was then used as the feed fiber to a second drawing stage on a pair of like drawing shoes at a draw ratio of 1.1:1 and a contact time of about .4 second as shown in Table III.

As can be seen from the data of Table IV, the less severe conditions used in the second stage draw treatment yield a polybenzimidazole fiber of increased tensile properties (i.e. tenacity and initial modulus). In Experiment Nos. 1 and 2 the temperature of the second stage draw treatment was excessive, and resulted in a decrease in the tenacity and initial modulus values. Experiment Nos. 3 and 4 indicate that both the tenacity and the initial modulus were enhanced in accordance with applicants' improved process.

As will be apparent to those skilled in the art, variations and modifications may be resorted to which depart from the specific conditions employed in the examples. Such variations and modifications are to be considered

TABLE III

| Experiment Number                            | Residence time in seconds | Draw ratio | Supply roll rate, meters/minute | Temperature in degrees centigrade | Denier per fiber | Elongation, percent | Tenacity, grams/denier | Initial modulus, grams/denier |
|----------------------------------------------|---------------------------|------------|---------------------------------|-----------------------------------|------------------|---------------------|------------------------|-------------------------------|
| I. Feed fiber from first draw                |                           |            |                                 |                                   |                  |                     |                        |                               |
|                                              | 0.7                       | 3.0        | 25                              | 430                               | 4.6              | 20.5                | 5.2                    | 23.4                          |
| II. Second stage draw conditions and results |                           |            |                                 |                                   |                  |                     |                        |                               |
| 1-----                                       | 0.4                       | 1.1        | 75                              | 445                               | 3.4              | 24.6                | 4.5                    | 22.3                          |
| 2-----                                       | 0.4                       | 1.1        | 75                              | 430                               | 3.4              | 22.7                | 5.1                    | 24.2                          |
| 3-----                                       | 0.4                       | 1.1        | 75                              | 415                               | 3.5              | 22.0                | 5.0                    | 23.5                          |
| 4-----                                       | 0.4                       | 1.1        | 75                              | 400                               | 3.3              | 15.4                | 5.7                    | 22.2                          |
|                                              |                           |            |                                 |                                   |                  |                     |                        | 102                           |

As can be seen from the data of Table III, the less severe conditions used in the second stage draw treatment yield a polybenzimidazole fiber of generally increased tensile properties (i.e. tenacity and initial modulus). In Experiment Nos. 1 and 2 the temperature of the second draw treatment was excessive. In Experiment No. 4 which was conducted in accordance with applicants'

within the scope and purview of the claims appended hereto.

We claim:

1. A process for improving the tensile properties of polybenzimidazole fiber, which comprises subjecting said fiber to a first draw treatment at a temperature in the range of from 300 to 650° C. and at a draw ratio in

the range of from 1.5:1 to 3.5:1, and thereafter subjecting the resulting drawn fiber to a second draw treatment at a draw ratio in the range of from 1.05:1 to 1.5:1 and at a temperature which is lower than that used in the first draw and which is within the range of from 200 to 500° C. to produce a polybenzimidazole fiber product having a higher tenacity and higher initial modulus than that of the fiber product obtained from said first draw treatment.

2. A process according to claim 1 wherein said polybenzimidazole fiber is an aromatic polybenzimidazole fiber.

3. A process according to claim 1 wherein said polybenzimidazole is poly-2,2'-(m-phenylene)-5,5'-bibenzimidazole.

4. A process according to claim 1 wherein said first draw is conducted via radiation heating for a period of time in the range of from 5 to 30 seconds at a draw ratio of from 2.0:1 to 3.2:1, and said second draw treatment is conducted via radiation heating for a period of time in the range of from 1 to 20 seconds at a draw ratio of from 1.1:1 to 1.3:1.

5. A process according to claim 1 wherein said first draw is conducted via conduction heating for a period of time in the range of from 0.2 to 3 seconds, and said second draw treatment is conducted via conduction heating for a period of time in the range of from 0.1 to 1.5 seconds at a draw ratio of from 1.1:1 to 1.3:1.

6. A process according to claim 2 wherein said resulting draw fiber from said first draw treatment is subjected to a second draw treatment at a lower temperature, residence time and draw ratio than employed in said first draw treatment.

7. A process for improving the tensile properties of polybenzimidazole fiber, which comprises subjecting said fiber to a first draw treatment via radiation heating at a temperature in the range of from 450 to 600° C. for a period of time of from 5 to 30 seconds at a draw ratio

of from 1.5:1 to 3.5:1, and thereafter subjecting the resulting drawn fiber to a second draw treatment via radiation heating at a lower temperature than the first draw which is within the range of from 390 to 470° C. for a period of from 1 to 20 seconds at a draw ratio of from 1.05:1 to 1.5:1 to produce a polybenzimidazole fiber product having a higher tenacity and higher initial modulus than that of the fiber product obtained from said first draw treatment.

8. A process according to claim 7 wherein said polybenzimidazole fiber is an aromatic polybenzimidazole fiber.

9. A process according to claim 7 wherein said polybenzimidazole is poly-2,2'-(m-phenylene)-5,5'-bibenzimidazole.

10. A process according to claim 7 wherein said first stage draw treatment is conducted at a draw ratio of from 2.0:1 to 3.2:1, and said second stage draw treatment is conducted at a draw ratio of from 1.1:1 to 1.3:1.

11. A process according to claim 10 wherein said resulting drawn fiber from said first draw treatment is subject to a second draw treatment at a lower temperature, residence time and draw ratio than employed in said first draw treatment.

#### References Cited

##### UNITED STATES PATENTS

|           |         |                |       |           |
|-----------|---------|----------------|-------|-----------|
| 3,400,192 | 9/1968  | Hartmann       | ----- | 264—290 T |
| 3,441,640 | 4/1969  | Santangelo     | ----- | 264—203   |
| 3,526,693 | 9/1970  | Rulison et al. | ----- | 264—290 R |
| 3,541,199 | 11/1970 | Bohrer et al.  | ----- | 264—290 R |
| 3,584,104 | 6/1971  | Bohrer et al.  | ----- | 264—290 R |

HERBERT MINTZ, Assistant Examiner

U.S. Cl. X.R.

264—204